

# United States Patent

Motoyuki

[15] 3,650,817

[45] Mar. 21, 1972

[54] **METHOD OF MANUFACTURING LOW THERMAL-EXPANSION PORCELAIN**

[72] Inventor: Inoue Motoyuki, Nagoya-shi, Japan

[73] Assignee: Nippon Toki Kabushiki Kaisha, Nagoya-shi, Aichi-ken, Japan

[22] Filed: Aug. 8, 1969

[21] Appl. No.: 848,693

**Related U.S. Application Data**

[63] Continuation-in-part of Ser. No. 499,022, Oct. 20, 1965, Pat. No. 3,499,787.

[52] U.S. Cl..... 117/118, 65/33, 65/62, 106/45, 106/46, 106/48, 117/125

[51] Int. Cl..... C03c 17/00

[58] Field of Search ..... 65/33, 62; 117/118, 124, 125, 117/169; 106/39, 45, 46, 48

[56] **References Cited**

**UNITED STATES PATENTS**

|           |         |                |          |
|-----------|---------|----------------|----------|
| 2,662,826 | 12/1953 | Schuepp .....  | 106/45   |
| 2,741,008 | 4/1956  | Snoddy .....   | 106/45 X |
| 2,919,995 | 1/1960  | Landron .....  | 106/65 X |
| 3,019,116 | 1/1962  | Doucetto ..... | 106/48 X |

|           |         |                       |           |
|-----------|---------|-----------------------|-----------|
| 3,170,805 | 2/1965  | McMillan et al.....   | 106/48 X  |
| 3,423,217 | 1/1969  | Blaha .....           | 106/48 X  |
| 3,449,203 | 6/1969  | Fischer .....         | 106/48 X  |
| 3,458,331 | 7/1969  | Kroger .....          | 106/45    |
| 3,480,452 | 11/1969 | Fleischner et al..... | 106/48 X  |
| 3,499,787 | 3/1970  | Inowe .....           | 117/125 X |
| 3,501,321 | 3/1970  | Margola.....          | 106/45    |

**FOREIGN PATENTS OR APPLICATIONS**

239,249 7/1962 Australia .....

*Primary Examiner—William D. Martin*

*Assistant Examiner—M. R. Lusignan*

*Attorney—Stevens, Davis, Miller & Mosher*

[57] **ABSTRACT**

A heat resistant porcelain body having a smooth, dense and hard glaze layer on the surface thereof is prepared by coating a porcelain body comprised of at least one of petalite and spodumene in admixture with plastic clay and containing specified amounts of  $Al_2O_3$ ,  $SiO_2$  and  $LiO_2$  in addition to at least one of 0.5-6 percent by weight of  $ZnO$  and 7-26 percent by weight of free  $SiO_2$  with a glaze preparation containing primarily  $SiO_2$  and thereafter firing the coated porcelain body at 1250°-1350° C.

**6 Claims, No Drawings**

## METHOD OF MANUFACTURING LOW THERMAL-EXPANSION PORCELAIN

This application is a continuation-in-part of application Ser. No. 499,022, filed Oct. 20, 1965, now U.S. Pat. No. 3,499,787, dated March 10, 1970.

This invention relates to a process for manufacturing a heat-resistant porcelain body having a smooth, dense and hard glaze layer on the surface thereof, the porcelain body having a low thermal-expansion coefficient which is more especially, in the range of from  $3.9 \times 10^{-6}$  to 0.

Hitherto, a great difficulty has been experienced in attempting to coat the surface of a porcelain body having a low coefficient of thermal-expansion with a glaze having a still lower coefficient of thermal-expansion than that of the porcelain body. For such glazing purposes, various attempts have been made including coating with very thin glassy layers, self-glazing and cracked glazing, but none has proved satisfactory.

The formation of thin glassy films involves difficulties in insuring uniform thickness and tends to cause cracks in thick portions of the film. Self-glazing is quite susceptible to variations in heating or cooling conditions and the glazing process makes it difficult and impracticable to obtain products of stable qualities. Cracked glazing also has the disadvantages, in that the tensile stress due to the difference in coefficient of thermal-expansion between the glaze and the body is exerted on the surface of the porcelain body to lower the thermal shock resistance producing cracks, which tend to collect impurities leading to sanitation problems and inferior appearance.

An object of this invention is to provide a porcelain body having a low coefficient of thermal-expansion with a glaze layer having a low coefficient of thermal-expansion.

Another object of this invention is to provide a porcelain body with a smooth, dense, hard, and crack-free glaze layer which has a low coefficient of thermal-expansion.

A further object of this invention is to provide a process for manufacturing a porcelain body which possesses the aforesaid characteristics.

According to the present invention there is provided a process for manufacturing a porcelain body having a low coefficient of thermal-expansion and being provided with a smooth, dense and hard glaze layer thereon, which comprises (a) coating a porcelain body with a glaze-forming material, the composition of said porcelain body and the glaze-forming material being such that when the coating of the glaze-forming material applied to said porcelain body is heated, components of said porcelain body and glaze-forming material react with each other during the heating thereof to form, in the glaze, 50 crystals having a low coefficient of thermal-expansion and (b) heating the coated porcelain body to vitrify and simultaneously to produce a quantity of said crystals having a low thermal-expansion coefficient in the glaze, whereby, on cooling a smooth, dense and hard glaze layer is formed on the porcelain body.

Thus, the objects of the invention are accomplished by (a) coating a green or biscuit body surface of porcelain with a glaze-forming material which will react with the main constituents or additives of the body to form crystals of low thermal-expansion coefficient in the glaze, and (b) firing the coated body to vitrify and also to form a glaze layer which contains a substantial amount of crystals with a low coefficient of thermal-expansion on the surface of said porcelain body, thereby on cooling obtaining a smooth, dense, and hard porcelain which is also non-porous and possesses a good thermal shock resistance.

Specifically, in order to obtain the above desired objectives, a porcelain body is made up of a composition comprising at least one mineral selected from the group consisting of petalite and spodumene in admixture with plastic clay, preferably kaolin. When using petalite it should be employed in an amount of about 40-90 percent by weight with the clay being present in an amount of about 10-60 percent by weight. When using spodumene this should be employed in an amount

of 30-60 percent by weight with the clay being about 40-70 percent by weight. The mixture should contain 55-74 percent by weight of  $\text{SiO}_2$ , 18-32 percent by weight of  $\text{Al}_2\text{O}_3$  and about 1.5-4.5 percent by weight of  $\text{Li}_2\text{O}$ . When spodumene and petalite are used in admixture their relative proportions can vary widely, it being only necessary that the content of  $\text{Li}_2\text{O}$  derived from the petalite and spodumene comprise about 1.5-4.5 percent by weight of the body composition. These proportions, of course, are easily calculated from the known  $\text{Li}_2\text{O}$  content of spodumene and petalite which are listed hereinafter. Normally the composition will also contain small amounts of  $\text{K}_2\text{O}$  and  $\text{Na}_2\text{O}$ , e.g., 1-3 percent since these later oxides are normally present in the lithium aluminum silicates known as petalite and spodumene and in plastic clay. The ignition loss of the composition will usually be between 1.5 and 11 percent by weight, after firing.  $\text{K}_2\text{O}$  and  $\text{Na}_2\text{O}$ , however, are not essential constituents.

It is necessary to produce large quantities of low thermal-expansion crystals in the glaze-forming material in order that the resulting glaze layer is suitable as such for the low thermal-expansion porcelain body on which it is formed. If a body containing  $\text{Li}_2\text{O}$  in a large amount, such as a petalite-clay or spodumene-clay body, is coated with a glaze-forming material 15 and then fired, a large amount of  $\text{Li}^+$  ions will be diffused from the body to the glaze-forming material to promote the fusion thereof and consequently hinder the glaze-forming material from crystallizing, thereby making it impossible for the resulting glaze layer to have low thermal-expansion property. In order to solve this problem, it is necessary that the body contains free silica in amounts of 7-26 percent. If the original body contains less than 7 percent of free silica, additional free silica must be incorporated, as an additive, in the original body to the extent that it contains at least 7 percent of free silica, or else 0.5-6 percent of  $\text{ZnO}$  must be added to the original body. However, the use of more than 26 percent of free silica in the body will increase the thermal-expansion coefficient of the fired body and deteriorate the heat resistance of the porcelain product so obtained. The addition of 30 more than 6 percent of  $\text{ZnO}$  to the body is undesirable because this will cause the firing temperatures to be lowered and a deformed fired body to be produced.

The constituents of the composition discussed above are 35 products of nature, the principal composition of which is as follows:

|           |              |                                                  |        |
|-----------|--------------|--------------------------------------------------|--------|
| Petalite  | Plastic clay | : Ig loss                                        | 13-15% |
|           |              | : $\text{SiO}_2$                                 | 48-51% |
|           |              | : $\text{Al}_2\text{O}_3$                        | 31-33% |
| Spodumene |              | : $\text{K}_2\text{O} \cdot \text{Na}_2\text{O}$ | 1-3%   |
|           |              | : $\text{SiO}_2$                                 | 75-77% |
|           |              | : $\text{Al}_2\text{O}_3$                        | 15-17% |
| Kaolin    |              | : $\text{Li}_2\text{O}$                          | 3-4%   |
|           |              | : $\text{K}_2\text{O} \cdot \text{Na}_2\text{O}$ | 1%     |
|           |              | : $\text{SiO}_2$                                 | 60-63% |
|           |              | : $\text{Al}_2\text{O}_3$                        | 27-30% |
|           |              | : $\text{Li}_2\text{O}$                          | 6-7%   |
|           |              | : $\text{Na}_2\text{O} \cdot \text{K}_2\text{O}$ | 1-2%   |
|           |              | : Ig loss                                        | 11-14% |
|           |              | : $\text{SiO}_2$                                 | 45-48% |
|           |              | : $\text{Al}_2\text{O}_3$                        | 35-38% |
|           |              | : $\text{K}_2\text{O} + \text{Na}_2\text{O}$     | 1-2%   |

As is seen from the above, there is some variation in the amount of the individual compounds of each of the minerals petalite and spodumene and clay. Therefore, it will be seen that the specific amount of petalite or spodumene within the percentages recited above which are listed with the plastic clay within the recited percentages must be such that the amounts of the critical constituents  $\text{SiO}_2$ ,  $\text{Al}_2\text{O}_3$  and  $\text{Li}_2\text{O}$  fall within the ranges set forth above when the composition is prepared. The plastic clay such as kaolin also contributes quantities of  $\text{SiO}_2$  and  $\text{Al}_2\text{O}_3$  which amounts are to be included within the percentages set forth. The amount of the mixture of the minerals (petalite and spodumene) and the clay in the porcelain body should constitute about 74-99.5 percent by weight of the body.

An essential feature of the present invention is that there be included in the porcelain body certain additives, namely zinc oxide in an amount of 0.5-6 percent, preferably 2-5 percent, based on the total weight of the porcelain body and/or free  $\text{SiO}_2$  in an amount of 5-20 percent, preferably 7-15 percent by weight based on the total weight of the porcelain body. It is to be noted that the additive-incorporated porcelain body contains free  $\text{SiO}_2$  in amounts of 7-26 percent by weight because the original body contains  $\text{SiO}_2$  in amounts of 2-6 percent by weight.

By including these additives in the indicated amounts, the objectives of the present invention are achieved by virtue of reaction between the components of the body and the components of the glaze composition which will be hereinafter described in order to form a substantial amount of crystals within the glaze having a low thermal coefficient of expansion and composed principally of Silica O solid solution crystals whose end members are composed of  $\beta$ -quartz and  $\beta$ -eucryptite, or  $\beta$ -spodumene solid solution crystals.

Though the porcelain body coated according to the process of this invention has been defined in terms of its essential ingredients, namely the mineral, the plastic clay, e.g., kaolin, and the additives  $\text{ZnO}$  and/or free  $\text{SiO}_2$  it must be recognized that minor amounts of conventional additives for the promotion of vitrification or for the extension of the firing temperature range may also be present, for example, the oxides, carbonates or silicates of barium, magnesium, calcium, strontium and lead as well as feldspar, nepheline and talc. Normally these additives will make up less than 5 percent of the total porcelain body. The actual formation of the porcelain body is conducted in a conventional manner, utilizing the well known jiggering or casting methods.

According to the next step of the instant process, the surface of the formed green body or its biscuit is coated with a glaze preparation comprising 60-79 percent  $\text{SiO}_2$ ; 9-12 percent  $\text{Al}_2\text{O}_3$ ; 0-20 percent  $\text{ZnO}$ ; 0-7 percent  $\text{MgO}$ ; 2-5 percent  $\text{CaO}$ ; 0-7 percent  $\text{Li}_2\text{O}$  (all molar percentages) and traces of  $\text{K}_2\text{O}$  and  $\text{Na}_2\text{O}$  and other compounds. The application of the glaze to the green body or biscuit is also a conventional step involving preparation of an aqueous slurry of the finely divided glaze constituents and application thereof to the surface of the green or biscuit body. The coated body is then fired at 1250°-1350° C. whereby the coated body is vitrified and simultaneously the glaze layer is formed containing a large amount of Silica O or  $\beta$ -spodumene solid solution crystals. Various oxides of the glaze preparation listed above are conveniently added in the form of natural existing minerals or clays. Thus, for example, the glaze composition may include silica sand, calcined kaolin, alkaline feldspar, alumina, petalite, talc, dolomite, limestone and zinc oxide. These materials which may be used in the preparation of the glaze are composed principally as follows:

|                                          |   |                                   |        |
|------------------------------------------|---|-----------------------------------|--------|
| Silica Sand                              | : | $\text{SiO}_2$                    | 94-97% |
|                                          |   | $\text{Al}_2\text{O}_3$           | 1-2%   |
|                                          |   | $\text{K}_2\text{O Na}_2\text{O}$ | 1-2%   |
| Alkaline feldspar                        | : | $\text{SiO}_2$                    | 65-67% |
|                                          |   | $\text{Al}_2\text{O}_3$           | 16-18% |
|                                          |   | $\text{K}_2\text{O Na}_2\text{O}$ | 12-14% |
| Petalite                                 | : | $\text{SiO}_2$                    | 75-77% |
|                                          |   | $\text{Al}_2\text{O}_3$           | 15-17% |
|                                          |   | $\text{Li}_2\text{O}$             | 3-4%   |
|                                          |   | $\text{K}_2\text{O Na}_2\text{O}$ | 1%     |
| Kaolin (calcined)                        | : | $\text{SiO}_2$                    | 54-56% |
|                                          |   | $\text{Al}_2\text{O}_3$           | 38-42% |
|                                          |   | $\text{K}_2\text{O Na}_2\text{O}$ | 2-3%   |
| Alumina                                  | : | $\text{Al}_2\text{O}_3$           | 99%    |
| Talc (calcined)                          | : | $\text{SiO}_2$                    | 65-67% |
|                                          |   | $\text{MgO}$                      | 32-34% |
| Dolomite (A calcium magnesium carbonate) | : | $\text{CaMg}(\text{Co}_3)$        |        |
|                                          |   | Ig loss                           | 44-47% |
|                                          |   | $\text{CaO}$                      | 32-35% |
|                                          |   | $\text{MgO}$                      | 17-20% |
| Limestone                                | : | Ig loss                           | 43-45% |
|                                          |   | $\text{CaO}$                      | 54-57% |
| Zinc white                               | : | $\text{ZnO}$                      | 98%    |

The coefficient of thermal-expansion of the glaze can be varied over a broad range of  $3.9 \times 10^{-6}$ -0 by controlling the amounts of  $\text{ZnO}$ ,  $\text{SiO}_2$  and  $\text{Li}_2\text{O}$  in the body without further treatment such as reheating.

5 A low thermal-expansion porcelain thus obtained has a smooth, dense, and hard glazed surface and is non-porous. Therefore it has a good appearance as well as durability which makes this porcelain suitable and useful for tableware and industrial applications. Furthermore, it will possess thermal 10 shock-resistance and physical strength because of the great compressive stress in the glaze.

In order to more clearly illustrate the present invention, the following examples are presented:

15

### EXAMPLE 1

A petalite clay composition consisting of:

| Total Analysis |           |                                          |            |
|----------------|-----------|------------------------------------------|------------|
| 20 Petalite    | 44% (wt.) | Ignition loss                            | 6.8% (wt.) |
|                |           | $\text{SiO}_2$                           | 61.8       |
| Plastic clay   | 45% (wt.) | $\text{Al}_2\text{O}_3$                  | 22.5       |
|                |           | $\text{Li}_2\text{O}$                    | 1.8        |
| Zinc white     | 6% (wt.)  | $\text{K}_2\text{O}+\text{Na}_2\text{O}$ | 1.0        |
|                |           | $\text{ZnO}$                             | 6.0        |
| 25 Silica Sand | 5% (wt.)  | Others                                   | 0.1        |

is finely ground and mixed by ball mill. Ferrous contents and excess water are removed from the mixture. The mixture is then formed to a porcelain body by casting.

30 Next, a green glaze composition consisting of

| Total Analysis  |           |                                          |              |
|-----------------|-----------|------------------------------------------|--------------|
| 35 Silica sand  | 43% (wt.) | $\text{SiO}_2$                           | 77.6% (mol.) |
| Alumina         | 11% (wt.) | $\text{Al}_2\text{O}_3$                  | 9.4% (mol.)  |
|                 |           | $\text{CaO}$                             | 2.4% (mol.)  |
| Petalite        | 20% (wt.) | $\text{MgO}$                             | 6.7% (mol.)  |
|                 |           | $\text{K}_2\text{O}+\text{Na}_2\text{O}$ | 2.4% (mol.)  |
| Feldspar        | 13% (wt.) | $\text{Li}_2\text{O}$                    | 1.8% (mol.)  |
| Talc (calcined) | 7% (wt.)  |                                          |              |
| Dolomite        | 6% (wt.)  |                                          |              |

40 is finely ground and mixed by ball mill and applied on the surface of the above green or biscuit body. The coated body is then fired at 1250°-1300° C.

The characteristics of the product thus obtained are as follows:

|                                                                      |   |                          |
|----------------------------------------------------------------------|---|--------------------------|
| 45 Bending strength                                                  | : | 650 kg./cm. <sup>2</sup> |
| Linear thermal-expansion coefficient (porcelain body) (at 0-600° C.) | : | $2.5 \times 10^{-6}$     |
| 50 Linear thermal-expansion coefficient (glaze) (at 0-600° C.)       | : | $2.2 \times 10^{-6}$     |
| Thermal shock resistance (quenching temp. dif.)                      | : | 360° C.                  |
| Color                                                                | : | white                    |
| Surface condition                                                    | : | mat, dense, and hard     |

55

### EXAMPLE 2

A porcelain product is obtained in the same manner as in Example 1, using a petalite-clay body composition consisting of:

| Total Analysis |           |                                          |             |
|----------------|-----------|------------------------------------------|-------------|
| 65 Petalite    | 65% (wt.) | Ignition loss                            | 3.3% (wt.)  |
|                |           | $\text{SiO}_2$                           | 71.0% (wt.) |
| Plastic clay   | 22% (wt.) | $\text{Al}_2\text{O}_3$                  | 18.6% (wt.) |
|                |           | $\text{Li}_2\text{O}$                    | 2.6% (wt.)  |
| Zinc white     | 3% (wt.)  | $\text{K}_2\text{O}+\text{Na}_2\text{O}$ | 1.0% (wt.)  |
|                |           | $\text{ZnO}$                             | 3.0% (wt.)  |
| Silica sand    | 10% (wt.) | Others                                   | 0.5% (wt.)  |

70 and a green glaze composition consisting of:

| Total Analysis    |           |                                          |              |
|-------------------|-----------|------------------------------------------|--------------|
| 75 Silica sand    | 10% (wt.) | $\text{SiO}_2$                           | 69.5% (mol.) |
| Kaolin (calcined) | 18% (wt.) | $\text{Al}_2\text{O}_3$                  | 11.3% (mol.) |
| Petalite          | 55% (wt.) | $\text{CaO}$                             | 2.7% (mol.)  |
|                   |           | $\text{K}_2\text{O}+\text{Na}_2\text{O}$ | 0.9% (mol.)  |

|            |          |                   |             |
|------------|----------|-------------------|-------------|
| Limestone  | 4%(wt.)  | Li <sub>2</sub> O | 4.9%(mol.)  |
| Zinc white | 13%(wt.) | ZnO               | 10.7%(mol.) |

The porcelain product so obtained has the following characteristics:

|                                                                      |                            |
|----------------------------------------------------------------------|----------------------------|
| Bending strength                                                     | : 600 kg./cm. <sup>2</sup> |
| Linear thermal-expansion coefficient (porcelain body) (at 0-600° C.) | : $0.8 \times 10^{-6}$     |
| Linear thermal-expansion coefficient (glaze) (at 0-600° C.)          | : $0.3 \times 10^{-6}$     |
| Thermal shock resistance (quenching temp. dif.)                      | : 600° C.                  |
| Color                                                                | : White                    |
| Surface condition                                                    | : Mat, dense, and hard     |

### EXAMPLE 3

Following the procedure of Example 1 but using a petalite-clay composition consisting of:

| Total Analysis |          |                                    |             |
|----------------|----------|------------------------------------|-------------|
| Petalite       | 70%(wt.) | Ignition loss                      | 4.1%(mol.)  |
| Plastic clay   | 27%(wt.) | SiO <sub>2</sub>                   | 67.7%(mol.) |
| Zinc white     | 3%(wt.)  | Al <sub>2</sub> O <sub>3</sub>     | 20.8%(mol.) |
|                |          | Li <sub>2</sub> O                  | 2.8%(mol.)  |
|                |          | K <sub>2</sub> O+Na <sub>2</sub> O | 1.0%(mol.)  |
|                |          | ZnO                                | 3.0%(mol.)  |
|                |          | Others                             | 0.6%(mol.)  |

and a green glaze composition consisting of:

| Total Analysis    |          |                                    |             |
|-------------------|----------|------------------------------------|-------------|
| Silica sand       | 9%(wt.)  | SiO <sub>2</sub>                   | 70.1%(mol.) |
| Kaolin (calcined) | 17%(wt.) | Al <sub>2</sub> O <sub>3</sub>     | 11.3%(mol.) |
| Petalite          | 58%(wt.) | CaO                                | 2.7%(mol.)  |
| Limestone         | 4%(wt.)  | K <sub>2</sub> O+Na <sub>2</sub> O | 0.9%(mol.)  |
| Zinc white        | 12%(wt.) | Li <sub>2</sub> O                  | 5.2%(mol.)  |
|                   |          | ZnO                                | 9.9%(mol.)  |

is obtained a porcelain product which has the following characteristics:

|                                                                      |                            |
|----------------------------------------------------------------------|----------------------------|
| Bending strength                                                     | : 600 kg./cm. <sup>2</sup> |
| Linear thermal-expansion coefficient (porcelain body) (at 0-600° C.) | : $0.2 \times 10^{-6}$     |
| Linear thermal-expansion coefficient (glaze) (at 0-600° C.)          | : 0.0                      |
| Thermal shock resistance (temp. difference)                          | : 620° C.                  |
| Color                                                                | : White                    |
| Surface condition                                                    | : Mat, dense and hard      |

### EXAMPLE 4

There is obtained a porcelain product in the same manner in Example 1, using a petalite-clay body composition consisting of:

| Total Analysis |          |                                |            |
|----------------|----------|--------------------------------|------------|
| Petalite       | 85%(wt.) | Ignition loss                  | 2.1%(wt.)  |
| Plastic clay   | 14%(wt.) | SiO <sub>2</sub>               | 72.6%(wt.) |
| Zinc white     | 1%(wt.)  | Al <sub>2</sub> O <sub>3</sub> | 19.1%(wt.) |

and a green glaze composition consisting of:

| Total Analysis    |          |                                |             |
|-------------------|----------|--------------------------------|-------------|
| Silica sand       | 6%(wt.)  | SiO <sub>2</sub>               | 72.8%(mol.) |
| Kaolin (calcined) | 12%(wt.) | Al <sub>2</sub> O <sub>3</sub> | 11.0        |
| Petalite          | 70%(wt.) | CaO                            | 2.0         |

Limestone

Zinc white

5 3,650,817 6

The porcelain product so obtained has the following characteristics:

|    |                                                                      |                            |
|----|----------------------------------------------------------------------|----------------------------|
| 5  | Bending strength                                                     | : 550 kg./cm. <sup>2</sup> |
|    | Linear thermal-expansion coefficient (porcelain body) (at 0-600° C.) | : $0.2 \times 10^{-6}$     |
| 10 | Linear thermal-expansion coefficient (glaze) (at 0-600° C.)          | : 0.0                      |
|    | Thermal shock resistance (temp. difference)                          | : 620° C.                  |
|    | Color                                                                | : White                    |
|    | Surface condition                                                    | : Mat, dense and hard      |

15

### EXAMPLE 5

Following the procedure of Example 1 but using a spodumene-clay composition consisting of:

| Total Analysis |          |                                    |            |
|----------------|----------|------------------------------------|------------|
| Spodumene      | 40%(wt.) | Ignition loss                      | 7.5%(wt.)  |
| Plastic clay   | 50%(wt.) | SiO <sub>2</sub>                   | 55.1%(wt.) |
| Zinc white     | 5%(wt.)  | Al <sub>2</sub> O <sub>3</sub>     | 28.2%(wt.) |
| Silica sand    | 5%(wt.)  | Li <sub>2</sub> O                  | 2.8%(wt.)  |
|                |          | K <sub>2</sub> O+Na <sub>2</sub> O | 1.4%(wt.)  |
|                |          | ZnO                                | 5.0%(wt.)  |

and a green glaze composition consisting of:

| Total Analysis     |          |                                    |             |
|--------------------|----------|------------------------------------|-------------|
| Silica sand        | 21%(wt.) | SiO <sub>2</sub>                   | 78.7%(mol.) |
| Alumina            | 4%(wt.)  | Al <sub>2</sub> O <sub>3</sub>     | 9.9%(mol.)  |
| Petalite           | 60%(wt.) | CaO                                | 1.6%(mol.)  |
| Feldspar           | 8%(wt.)  | MgO                                | 3.2%(mol.)  |
| 35 Talc (calcined) | 4%(wt.)  | K <sub>2</sub> O+Na <sub>2</sub> O | 1.5%(mol.)  |
| Dolomite           | 3%(wt.)  | Li <sub>2</sub> O                  | 5.1%(mol.)  |

The porcelain product so obtained has the following characteristics:

|    |                                                                      |                            |
|----|----------------------------------------------------------------------|----------------------------|
| 40 | Bending strength                                                     | : 650 kg./cm. <sup>2</sup> |
|    | Linear thermal-expansion coefficient (porcelain body) (at 0-600° C.) | : $0.6 \times 10^{-6}$     |
| 45 | Linear thermal-expansion coefficient (glaze) (at 0-600° C.)          | : $0.4 \times 10^{-6}$     |
|    | Thermal shock resistance (temp. difference)                          | : 580° C.                  |
|    | Color                                                                | : White                    |
|    | Surface condition                                                    | : Mat, dense and hard      |

50

### EXAMPLE 6

Repeating the procedure of Example 1 but using a spodumene-clay body composition consisting of:

| Total Analysis |          |                                |            |
|----------------|----------|--------------------------------|------------|
| Spodumene      | 60%(wt.) | Ignition loss                  | 3.0%(wt.)  |
| Plastic clay   | 20%(wt.) | SiO <sub>2</sub>               | 67.0%(wt.) |
| Silica sand    | 20%(wt.) | Al <sub>2</sub> O <sub>3</sub> | 24.8%(wt.) |

and a green glaze composition consisting of:

| Total Analysis    |          |                                |             |
|-------------------|----------|--------------------------------|-------------|
| Silica sand       | 14%(wt.) | SiO <sub>2</sub>               | 62.9%(mol.) |
| Kaolin (calcined) | 27%(wt.) | Al <sub>2</sub> O <sub>3</sub> | 11.8%(mol.) |
| Petalite          | 33%(wt.) | CaO                            | 4.3%(mol.)  |

The porcelain product so obtained has the following characteristics:

|    |                  |                            |
|----|------------------|----------------------------|
| 75 | Bending strength | : 550 kg./cm. <sup>2</sup> |
|----|------------------|----------------------------|

Limestone

Zinc white

The porcelain product so obtained has the following characteristics:

|                                                                      |                        |
|----------------------------------------------------------------------|------------------------|
| Linear thermal-expansion coefficient (porcelain body) (at 0-600° C.) | : $1.5 \times 10^{-6}$ |
| Linear thermal-expansion coefficient (glaze) (at 0-600° C.)          | : 1.2                  |
| Thermal shock resistance (temp. difference)                          | : 520° C.              |
| Color                                                                | : Brownish white       |
| Surface condition                                                    | : Mat, dense and hard  |

## EXAMPLE 7

There is obtained a porcelain product in the same manner as in Example 1, using a petalite-spodumene-clay body composition consisting of:

|              |           | Total Analysis                     |             |
|--------------|-----------|------------------------------------|-------------|
| Petalite     | 50% (wt.) | Ignition loss                      | 3.8% (wt.)  |
|              |           | SiO <sub>2</sub>                   | 68.9% (wt.) |
| Spodumene    | 20% (wt.) | Al <sub>2</sub> O <sub>3</sub>     | 22.9% (wt.) |
|              |           | Li <sub>2</sub> O                  | 3.4% (wt.)  |
| Plastic clay | 25% (wt.) | K <sub>2</sub> O+Na <sub>2</sub> O | 1.0% (wt.)  |
| Silica sand  | 5% (wt.)  |                                    |             |

and a green glaze composition consisting of:

|                   |           | Total Analysis                     |              |
|-------------------|-----------|------------------------------------|--------------|
| Silica sand       | 9% (wt.)  | SiO <sub>2</sub>                   | 70.1% (mol.) |
|                   |           | Al <sub>2</sub> O <sub>3</sub>     | 11.3% (mol.) |
| Kaolin (calcined) | 17% (wt.) | CaO                                | 2.7% (mol.)  |
|                   |           | K <sub>2</sub> O+Na <sub>2</sub> O | 0.9% (mol.)  |
| Petalite          | 58% (wt.) | Li <sub>2</sub> O                  | 5.2% (mol.)  |
| Limestone         | 4% (wt.)  | ZnO                                | 9.9% (mol.)  |
| Zinc white        | 12% (wt.) |                                    |              |

The porcelain product so obtained has the following characteristics:

|                                                                      |                            |
|----------------------------------------------------------------------|----------------------------|
| Bending strength                                                     | : 600 kg./cm. <sup>2</sup> |
| Linear thermal-expansion coefficient (porcelain body) (at 0-600° C.) | : $0.3 \times 10^{-6}$     |
| Linear thermal-expansion coefficient (glaze)                         |                            |

|                                             |                       |
|---------------------------------------------|-----------------------|
| (at 0-600° C.)                              | : 0.0                 |
| Thermal shock resistance (temp. difference) | : 600° C.             |
| Color                                       | : Brownish white      |
| Surface condition                           | : Mat, dense and hard |

What is claimed is:

1. Process for manufacturing a porcelain body having a low coefficient of thermal-expansion and being provided with a smooth, dense and hard glaze layer, which comprises coating a porcelain body with a glaze preparation, said porcelain body being made up of about 74-99.5 percent of a composition consisting essentially of at least one mineral selected from the group consisting of petalite and spodumene, in admixture with plastic clay, the total composition containing about 55-74 percent by weight SiO<sub>2</sub>, about 18-32 percent by weight Al<sub>2</sub>O<sub>3</sub> and about 1.5-4.5 percent by weight Li<sub>2</sub>O, said porcelain body, including at least one additive selected from the group consisting of 0.5-6 percent by weight ZnO and 7-26 percent by weight free SiO<sub>2</sub>, said glaze preparation consisting essentially of 60-79 mol percent SiO<sub>2</sub>, 9-12 mol percent Al<sub>2</sub>O<sub>3</sub>, 0-20 mol percent ZnO, 0-7 mol percent MgO, 2-5 mol percent CaO and 0-7 mol percent Li<sub>2</sub>O, and thereafter firing said coated porcelain body at a temperature of about 1250°-1350° to vitrify said porcelain and produce in the glaze crystals having a low thermal-expansion coefficient.
2. A process according to claim 1 wherein said porcelain body composition consists essentially of about 40-90 percent petalite and about 10-60 percent by weight of plastic clay.
3. A process according to claim 1 wherein said porcelain body composition consists essentially of about 30-60 percent by weight of spodumene and about 40-70 percent by weight of plastic clay.
4. A process according to claim 1 wherein said plastic clay is kaolin.
5. A method according to claim 1 wherein zinc oxide in the porcelain body is used in an amount of 2-5 percent.
6. Method according to claim 1 wherein the free SiO<sub>2</sub> in the porcelain body is present in an amount of 7-15 percent.

\* \* \* \* \*